

F. C. OVERBURY,  
ORNAMENTAL ROOFING,  
APPLICATION FILED JULY 24, 1920.

1,418,456.

Patented June 6, 1922.



Inventor:  
Frederick C. Overture  
by Elbridge Dyer Attys.  
H. D. S.

# UNITED STATES PATENT OFFICE.

FREDERICK C. OVERBURY, OF HILLSDALE, NEW JERSEY, ASSIGNOR TO THE FLINT-KOTE COMPANY, OF BOSTON, MASSACHUSETTS, A CORPORATION OF MASSACHUSETTS.

## ORNAMENTAL ROOFING.

1,418,456.

Specification of Letters Patent. Patented June 6, 1922.

Application filed July 24, 1920. Serial No. 398,681.

*To all whom it may concern:*

Be it known that I, FREDERICK C. OVERBURY, a citizen of the United States, residing at Hillsdale, in the county of Bergen and State of New Jersey, have invented new and useful Improvements in Ornamental Roofing, of which the following is a specification.

The object of the present invention is to produce an ornamental roofing material, either in the form of sheets or of strips or slabs, in which each element has its surface lined or striped.

It is customary, in the manufacture of roofing, to coat the felt (which has been saturated or impregnated with asphalt or equivalent water-repellent compound) with a relatively high-melting-point asphalt, and, while the coating is plastic and adhesive, to partially embed therein crushed flaky slate of any suitable color; and it has been proposed to employ slate or grit of different colors, and to supply the same in parallel bands or stripes of contrasting colors.

In the present case, I propose to coat the sheet as usual and to apply a layer of crushed slate or grit to the coating, much as ordinarily, but to remove a portion of the coating so as to leave zones or bands which are uncoated and unsurfaced with the slate or grit, and then to apply a colored plastic water-repellent material to such uncoated zones, with the result that the surface of the sheet has bands or zones of slate, and intervening bands or zones of the colored water-repellent material. The sheet thus formed may be wound into a roll for shipment, so as to be subsequently laid flat on a roof, or it may be divided transversely into shingle strips or slabs. In the latter case, the strips or slabs are laid in overlapping rows and simulate shingles or tiles.

On the accompanying drawing,—

Figure 1 represents more or less conventionally and diagrammatically an apparatus for carrying out the process.

Figure 2 represents the comb for stripping the coating from the parallel zones of the sheet.

Figure 3 represents the rolls for applying the colored plastic coating to the uncoated zones.

Figure 4 represents the finished sheet.

Referring to said drawings, the roll of dry felt is shown at 10, and the sheet is

drawn therefrom through the saturating tank 11, which contains molten asphalt or its equivalent, and thence through squeeze rolls 12 to remove the surplus saturating compound. The sheet then passes under roll 13, over rolls 14 and 15 (the latter being termed by me the "bed roll"), then around roll 16, and around roll 17, whence it passes to the set of cooling or refrigerating rolls indicated as a whole at 18. As the sheet travels in its tortuous path from roll 13 to the cooling rolls, it is treated as will now be described. At 19 there is a smooth cylindrical coating roll which dips into a pan or trough 20, to which molten asphalt is delivered by a spout 21 from a reservoir tank 22. A distributing roll 23 is located between rolls 19 and 14, and receiving the asphalt from the former applies it to and spreads it on the face of the sheet from edge to edge thereof. The asphalt is soft and plastic, and now, by means of a comb 24, set above the bed roll 15, I plow or wipe off the asphalt from parallel zones, thus leaving the sheet with uncoated stripes to which slate or grit will not adhere to an appreciable extent. The sheet, with its parallel bands of adhesive coating, is now passed under a shower of crushed slate, grit or other crushed mineral material of the desired color—say, blue-black, green, red, brown or the like. This material is contained in a hopper 25 and is delivered thereto from a source of supply indicated at 26 through a conduit 27. In passing around the roll 16, the slate is embedded in the stripes of adhesive coating, the surplus being returned to the hopper 25, which is made flaring for this purpose. I now apply stripes of adhesive water-repellent material to the uncoated zones of the sheet, so as to fill the grooves formed therein by the comb and the application of slate to the coated zones. The water-repellent material may consist of wax tailings, stearin pitch, asphalt or the like, to which a suitable pigment may be added to give it the desired color. Red iron oxide or ground hematite ore gives to the material a desirable red or brown color. However, the coating may be of any color such as may be desired, so that a contrast will be made with the color of the crushed slate or other mineral which is partially embedded in the previously coated zones. This second adhesive

55

60

65

70

75

80

85

90

95

100

105

coating compound is delivered from a tank 28 through a spout 29 to a pan or trough 30, into which dips a roll 31. Between the roll 31 and that at 17, I locate a roll which has circumferential flanges equal in width to the uncoated zones on the sheet, so that the plastic compound carried up on the surface of the roll 31 will be transferred to the said previously uncoated zones, as the sheet 10 passes around roll 17. The transfer roll is shown at 32, and its circumferential ribs or flanges are indicated at 33, see Figure 3.

It will be understood, of course, that the coating compounds in tanks 22 and 28 are 15 kept in a hot molten state by any usual or suitable means, and that suitable power-transmitting devices are employed to effect the rotation of the various rolls, where such power rotation is desirable.

20 After being treated as hereinbefore described, and after passing through the cooling rolls 18, the sheet may be passed through a festooning mechanism, indicated conventionally at 34, and then delivered to a machine 35, by which the sheet is chopped or 25 severed into slabs or strips.

In Figure 2, the operation of the comb is

illustrated. The sheet is indicated in cross section at *a*, and the first coating at *b*. The comb 24 has teeth 241, which scrape off the 30 coating from the face of the sheet leaving grooves *c*. The comb is adjustable toward and from the roll 15.

In Figure 4, the finished sheet is shown conventionally. It has the mineral- or slate-surfaced parallel zones *d*, and the intervening zones *e* which are surfaced with the colored coating. When the sheet is severed on the transverse lines *x-x*, shingle strips or slabs are formed which may be 40 laid to produce the effect of shingles, tiles or other individual elements.

What I claim is:—

A roofing material comprising a fibrous waterproof foundation, having on its face 45 spaced parallel zones of asphalt, surfaced with crushed mineral, and intervening zones of a plastic colored waterproof compound, which contrasts in color with the mineral-surfaced zones.

50 In testimony whereof I have affixed my signature.

FREDERICK C. OVERBURY.